

July 19, 1927.

1,636,367

R. ILLEMANN  
PROCESS OF COATING CONCRETE PIPES AND HOLLOW BODIES  
WITH BITUMINOUS COMPOSITIONS  
Filed Jan. 15, 1926

Fig. 1.



Fig. 2.



Fig. 4.



Inventor.  
R. Illemann.  
by Fetherstonhaugh Co.  
Atrys.

## UNITED STATES PATENT OFFICE.

ROBERT ILLEMANN, OF GLASGOW, SCOTLAND.

## PROCESS OF COATING CONCRETE PIPES AND HOLLOW BODIES WITH BITUMINOUS COMPOSITIONS.

Application filed January 15, 1926. Serial No. 81,473.

It is known to manufacture concrete pipes and other hollow bodies from a composition of cement and sand, or any other suitable aggregate, by centrifugal action, i. e. by a spinning process, also to hand mould or cast such pipes or bodies when the concrete is in a liquid or semi-liquid condition.

My invention relates to a process and also to a composition of matter, for use in the process, whereby pipes or other hollow bodies made of concrete can be effectively coated or lined on the inner surface and also, if required, on the outer surface with a bituminous-stone flour coating.

The practice usually adopted, up till now, for making concrete pipes and lining them with a hot bituminous material is, first, to spin the pipes from cement and any suitable aggregate and stack them away for setting and hardening, which takes several weeks, perhaps months, before the necessary hardness is attained for the various water pressures which the pipes are required to resist when the pipes are in use.

The main difficulty and drawback up till now is that such concrete pipes, even if they are hard and it is intended to line them with an inner coating of a hot bituminous material, require a specially prepared inner surface characterized by keys and grooves made when the concrete is soft; or, otherwise, stone chips thrown in and partly embedded in the concrete so as to provide a rough inner surface on the pipe these chips serving, when the concrete is set, as keys to give a grip or hold, to a certain extent, for the hot bituminous substance.

I have found the foregoing practice is not only expensive but it is most unreliable for the reason that the dampness or moisture which is still present in the hard concrete renders it impossible for the hot bituminous substance to adhere closely and uniformly on the inner surface of the concrete pipe.

If it is sought to drive off the moisture from the concrete pipe by heat and at the same time allow the inserted hot bituminous mass to run freely in the pipe, then I find a fine dusty film is formed due to the cement being overheated or "killed" and this film of fine dust on the inner surface of the concrete pipe prevents the hot bituminous substance adhering and uniformly uniting to

the concrete so that there is not an effective combination of the concrete and the bituminous substance.

The object of my invention is to overcome these difficulties.

According to my invention I manufacture bituminously lined pipes or other hollow bodies of concrete by spinning a mass of concrete to form the body, introducing a quantity of cold, aqueous, liquid bituminous composition into the body while the latter is still wet, continuing the spinning of the body to distribute the composition over the interior surface of the body and thereafter allowing or causing the concrete and the bituminous composition to set simultaneously.

As a liquid bituminous composition I prefer to use one whose preparation is herein-after fully described.

In carrying out the invention I proceed as follows:—

I prepare a cold, aqueous bituminous waterproofing composition, before the concrete pipe is made, by first making a creamy mixture of stone, reduced by grinding, crushing, or otherwise, to a condition such as flour, powder or dust, (hereinafter referred to as "stone-flour") and water, and heating the same to boiling point and agitating it, and then adding bitumen in a liquid condition by pouring same into the aforesaid boiling mixture the boiling being kept up and the mixture kept in a state of constant agitation until the mass is brought to the consistency of a stiff paste. I then put the same amount of water into the mixture as has been evaporated by the boiling,

thinning it down further with water, according to requirements, and I continually stir and agitate the whole mass till it is cool. In making the composition I may use the stone-flour and the bitumen in the proportion of about, for example, 48 lbs. by weight of the stone-flour fluid to 18 lbs. by weight of bitumen and this proportion I may vary according to the specific gravity of the materials and the bitumen used.

I wish it to be understood that when I use the expression "stone-flour" in the specification and the claims appended I wish the same to cover and include stone reduced to a floury state; stony matter such as slate, or sand, in a similar state (the sand being

reduced to a state finer than its natural state); and plumbago or graphite. With these substances no contraction of the composition occurs on drying, which is an important consideration.

I then proceed to spin the concrete pipe and as soon as the pipe is spun and made and while still wet and moist I immediately pour several gallons of the cold, aqueous 10 bituminous composition inside the concrete pipe and continue the spinning thereby distributing the composition, specially prepared for the purpose, all over the inner surface of the concrete pipe by centrifugal action 15 and the composition will adhere and unite firmly with the wet concrete forming an even layer of bituminous composition on the inside thereof and rendering the pipe non-porous, waterproof and acid resisting and 20 ready for use when dry.

After the spinning and lining of the concrete pipes with the said bituminous composition is completed they are stacked away to dry and harden, the bituminous composition 25 and concrete binding together and setting and hardening simultaneously.

For lining such pipes if required with a hot bituminous mixture containing no water, I proceed as follows:—

30 I take one or more concrete pipes previously treated as aforesaid with a coating of the before described mixture, when they are hard and dry, and place them back on the spinning machine, or any other suitable revolving device, and I close up each end of the concrete pipes temporarily in such a manner as to prevent the hot bituminous composition from running out when poured into the concrete pipes.

40 It is advisable before the hot bituminous composition is poured in, to warm the interior of the pipe with hot air or similar means, in order to allow the hot bituminous composition to run freely and evenly and 45 prevent the sudden chilling of the same.

After the required quantity of the hot bituminous composition has been spun and distributed evenly in each pipe, the pipes can be quickly cooled down, from the outside, with cold water applied by a water 50 hose, or any other suitable means, the pipes being revolved all the time until the hot bituminous composition inside the pipes is cold and hard and has firmly adhered to 55 the first applied bituminous composition so as to form on the inside a hard black and glossy lining after which the pipes are ready for use.

The quantity and thickness of the hot 60 bituminous coating is made according to requirements and to the diameter of and the water pressure to be resisted by the concrete pipes.

Instead of natural bitumen in either of 65 the bituminous compositions mentioned, I

may use pitch, tar, or similar bituminous and resinous matters or waxes, and which I wish to be covered by and included in the term "bituminous composition".

To increase the internal strength of the whole concrete pipe I choose a bitumen of most tenacious consistency and increase the melting point of the bitumen by adding thereto small quantities of sulphur flour, or, instead of sulphur, I may use stone-flour, and then add so much sand or crushed stone, or any suitable aggregate, to the mixture, till it is of a thick liquid consistency when hot. I may also increase the strength and tenacity of the bitumen by placing a circular reinforcement or any other suitable metallic reinforcement at the inner surface of the finished concrete pipe and pour and spin the hot liquid bituminous composition on top of same combining and surrounding such reinforcement with the bituminous composition and the concrete, thereby considerably increasing the strength of the whole concrete pipe. The layer of the bituminous composition may be of the same thickness as or more than the thickness of the concrete.

The drawings annexed hereto show such a reinforced concrete pipe, Fig. 1 being a longitudinal section partly broken away and Fig. 2 a cross section, while Fig. 3 shows a piece of reinforcement. Fig. 4 is a perspective view of the pipe.

In the drawings *a* is the concrete, *b* the bituminous-stone lining and *c* the reinforcement. This reinforcement preferably consists of longitudinal members *d* consisting of flat metal, such as shown at *e*, Fig. 1, twisted into spiral formation, such as shown at *f*, same figure, these spirals *f* being secured to circumferential members *g* (which may be plain round rods bent to shape) by welding at the junctions. As will be seen at Fig. 2 the reinforcement is embedded in and covered over by the lining.

The procedure hereinbefore referred to as applicable for concrete pipes would obviously be suitable for other hollow bodies made of concrete.

The bituminous composition made as hereinbefore described is not an emulsion, but is a composition formed by the microscopic particles of stone dust or flour, held in a state of suspension in the water, constituting nuclei to and around which the bitumen when it is introduced clings in such manner as to form a multitude of bitumen-stone globule which, when the water is evaporated, automatically adhere together and during the boiling process form a wet pasty mass. In this way the mass forms a bituminous-stone composition to which water can be added as desired for thinning purposes.

As the composition dries and sets the bituminous globules bind themselves together and seal and close up the pores left by the

evaporation of the water, thereby forming a close, solid and elastic waterproof lining or coating.

Having now fully described my invention 5 what I claim and desire to secure by Letters Patent is:—

1. A process of making bituminously lined pipes or other hollow bodies of concrete consisting in spinning a mass of concrete to 10 form the body, introducing a quantity of cold and aqueous liquid bituminous composition while the concrete is still wet, continuing the spinning of the body to distribute the bituminous composition over the interior 15 surface of the body and thereafter allowing the concrete and bituminous composition to set simultaneously.

2. A process of making bituminously lined pipes or other hollow bodies of concrete consisting in spinning a mass of concrete to 20 form the body, introducing into the body while the concrete is still wet a quantity of cold, aqueous bituminous composition composed of a mixture of liquid bitumen with stone-flour 25 and water, continuing the spinning of the body to distribute the bituminous composition over the interior surface of the body, and thereafter allowing the concrete and bituminous composition to set simultaneously 30 and become dry and hard.

3. A process of making bituminously lined pipes or other hollow bodies of concrete consisting in spinning a mass of concrete to 35 form the body, mixing liquid bitumen with stone-flour and water in about the proportion of 18 pounds weight of bitumen to 48 pounds weight of stone-flour fluid, introducing a quantity of the said mixture into the concrete body while the latter is still wet, 40 continuing the spinning of the body to distribute the bituminous mixture over the interior surface of the body, and thereafter allowing the concrete and the bituminous mixture to set simultaneously.

4. A process of making bituminously lined pipes or other hollow bodies of concrete consisting in spinning a mass of concrete to 45 form the body, preparing a mixture of stone-flour and water, heating same to the boiling point, adding bitumen in a liquid condition, maintaining the mixture in a boiling condition until it assumes the form of a stiff paste, adding water to the mass and agitating till cool, introducing a quantity of the aforesaid cold, aqueous bituminous mixture into the concrete body while the latter is still wet, continuing the spinning of the body to distribute the mixture over its interior surface, and thereafter allowing the concrete and the bituminous mixture to set simultaneously 50 and become dry and hard.

5. A process of making bituminously lined pipes or other hollow bodies of concrete consisting in spinning a mass of concrete to 55 form the body, introducing a quantity of cold,

aqueous, liquid bituminous composition while the concrete is still wet, continuing the spinning of the body to distribute the bituminous composition over the interior surface of the body, allowing the concrete and bituminous 70 composition to set simultaneously, placing the hardened body on the spinning machine, introducing a quantity of a hot non-aqueous bituminous composition, spinning the body to distribute same and thereafter cooling 75 the body and lining, the lining applied cold serving as a key for the subsequent hot lining.

6. The process of making bituminously lined pipes or other hollow bodies of concrete consisting in spinning a mass of concrete to 80 form the body, preparing a mixture of stone-flour and water, heating same to the boiling point, adding bitumen in a liquid condition, maintaining the mixture in a boiling 85 condition until it assumes the form of a stiff paste, adding water to the mass and agitating till cool, introducing a quantity of the aforesaid cold, aqueous bituminous mixture into the concrete body while the latter 90 is still wet, continuing the spinning of the body to distribute the mixture over its interior surface, allowing the concrete and the bituminous mixture therein to set simultaneously, again placing the hardened body 95 on the spinning machine, introducing a quantity of a hot non-aqueous bituminous composition, spinning the body to distribute same and until the hot bituminous composition within the body is cold and hard and 100 has firmly adhered to the first applied bituminous composition and forms a hard black and glossy lining.

7. A process of making bituminously lined pipes or other hollow bodies of concrete consisting in spinning a mass of concrete to 105 form the body, introducing a quantity of cold, liquid, bituminous composition while the concrete is still wet, continuing the spinning of the body to distribute the cold bituminous composition over the interior surface of the body, allowing the concrete and the bituminous composition to set simultaneously, inserting a cylindrical reinforcement into the body, again placing the hardened body on the spinning machine, introducing a quantity of a hot non-aqueous bituminous composition, spinning the body to 110 distribute same over the reinforcement and until the hot bituminous composition within the body is cold and hard and has firmly adhered to the first applied bituminous composition and forms a hard black and glossy lining.

8. A process of making bituminously lined pipes or other hollow bodies of concrete consisting in spinning a mass of concrete to 115 form the body, preparing a mixture of stone-flour and water, heating same to the boiling point, adding bitumen in a liquid condition, 120

- 4
- maintaining the mixture in a boiling condition until it assumes the form of a stiff paste, adding water to the mass and agitating till cool, introducing a quantity of the aforesaid 5 cold bituminous mixture into the concrete body while the latter is still wet, continuing the spinning of the body to distribute the mixture over its interior surface, allowing the concrete and the bituminous mixture 10 therein to set simultaneously, inserting a cylindrical reinforcement into the body, again placing the hardened body on the spinning machine, introducing a quantity of a hot non-aqueous bituminous composition, 15 spinning the body to distribute same over the reinforcement and until the hot bituminous composition within the body is cold and hard and has firmly adhered to the first applied bituminous composition and forms a 20 hard black and glossy lining.
9. A bituminously lined pipe made by spinning a mass of concrete to form the pipe, introducing a quantity of cold, aqueous, liquid bituminous composition while the 25 concrete is still wet, continuing the spinning of the pipe to distribute the bituminous composition over the interior surface of the pipe and thereafter allowing the concrete and bituminous composition to set simultaneously.
- 30 10. A bituminously lined pipe made by spinning a mass of concrete to form the pipe, introducing a quantity of cold and aqueous liquid bituminous composition while the

concrete is still wet, continuing the spinning of the pipe to distribute the bituminous composition over the interior surface of the pipe, allowing the concrete and bituminous composition to set simultaneously, placing the hardened body on the spinning machine, introducing a quantity of a hot non-aqueous 35 bituminous composition, spinning the pipe to distribute same and thereafter cooling the pipe and lining, with water or otherwise, the lining applied cold serving as a key for the subsequent hot lining.

11. A bituminously lined pipe made by spinning a mass of concrete to form the pipe, introducing a quantity of cold aqueous and liquid bituminous composition while the concrete is still wet, continuing the spinning of 40 the pipe to distribute the cold bituminous composition over the interior surface of the pipe, allowing the concrete and the bituminous composition to set simultaneously, inserting a cylindrical reinforcement into 45 the pipe, again placing the hardened pipe on the spinning machine, introducing a quantity of a hot non-aqueous bituminous composition, spinning the pipe to distribute same over the reinforcement and until the 50 hot bituminous composition within the body is cold and hard and has firmly adhered to the first applied bituminous composition and forms a hard black and glossy lining.

In testimony whereof I affix my signature.  
ROBERT ILLEMANN.